

# UNITED STATES PATENT OFFICE.

MENTHEIM SALOMON, OF TOLEDO, OHIO, ASSIGNOR TO EDWARD A. DEWEY, OF TOLEDO, OHIO.

## FUEL.

No. 806,194.

Specification of Letters Patent.

Patented Dec. 5, 1905.

Application filed July 22, 1905. Serial No. 270,863.

*To all whom it may concern:*

Be it known that I, MENTHEIM SALOMON, a citizen of the German Empire, residing at Toledo, in the county of Lucas and State of Ohio, 5 have invented new and useful Improvements in Fuel, of which the following is a specification.

The object of this invention is to utilize as fuel coal which is too fine for burning in the ordinary way and in its natural state; and with this object in view comminuted coal is mixed with binding material and subjected to high pressure, whereby it is formed into extremely dense blocks of such size and form as may seem best for the proposed use whether it be for domestic or other purposes. Fuel of this general kind has been produced in a variety of ways and from widely-different ingredients; but, so far as I am aware, the product has not 10 been entirely satisfactory. It is essential that the cost of labor and material should be low, that the fuel should not melt and clog the fire nor disintegrate long before it is consumed, that the lumps should not be too soft nor too 15 brittle to resist rough handling, that the fuel should not deteriorate by lapse of time or the action of moisture, and that its odor in burning should not be offensive. It is desirable that it should not involve certain minor evils 20 and that it should possess certain positive characteristics tending to make it more satisfactory in use.

My fuel consists of compact blocks or lumps made up of comminuted coal, pine-pitch, glue, 25 and common brown sugar, and it is produced by boiling the glue with sufficient water to make a thin liquid, boiling the pitch separately, boiling both together until they are intimately mixed, adding the sugar and boiling the whole mass until it is homogeneous, 30 thoroughly mixing this mass with comminuted coal, and subjecting the compound to heavy

pressure in suitable molds to form it into lumps or blocks of either rounded or angular form and of a size suitable for the proposed 45 use to be made of it.

In practice I have found the following proportions quite satisfactory: coal, two thousand pounds; pine-pitch, thirty-five pounds; 50 glue, five pounds; sugar, two pounds.

The pitch serves as a binder, and it is greatly aided by the glue, which although small in quantity is very evenly distributed by means of the water. The sugar may also serve to some slight degree as a binder; but, so far as 55 I am able to determine, it does not do more in this respect than to retard disintegration of the lumps when burning. Its principal office, perhaps, in this compound is to prevent unpleasant odors in the burning of the fuel. 60

What I claim is—

1. The process of forming fuel-lumps which consists in dissolving glue in boiling water, adding boiling pitch, adding sugar and boiling the whole, intimately mixing the liquid 65 so formed with comminuted coal, and subjecting the mass to high pressure.

2. Fuel-lumps consisting of comminuted coal, pine-pitch, glue, and sugar.

3. A fuel in which pine-pitch and glue are 70 combined with sugar; whereby objectionable odor in burning is prevented.

4. Highly-compressed fuel-blocks consisting of comminuted coal, pine-pitch, glue, and common sugar, in substantially the proportions of: coal, two thousand pounds, pitch, thirty-five pounds, glue, five pounds, and sugar, two pounds. 75

In testimony whereof I affix my signature in presence of two subscribing witnesses.

MENTHEIM SALOMON.

Witnesses:

JOHN ROOT,

MICHAEL J. GAVIN.